

## UNITED STATES PATENT OFFICE

1,963,298

## WIRE DRAWING METHOD

Flint C. Elder, Cleveland Heights, Ohio, assignor  
to The American Steel and Wire Company of  
New Jersey, a corporation of New Jersey

No Drawing. Application July 23, 1929,  
Serial No. 380,469

7 Claims. (Cl. 205—21)

This invention relates to the manufacture of wire and rods, and while not limited thereto, relates more particularly to the manufacture of lubricated wire and rods which are primarily intended for reworking in the manufacture of rivets, bolts and similar articles which are cold worked in suitable dies and require a lubricated surface.

Heretofore various lubricants such as oils and greases have been used to lubricate the wire and rods prior to their being worked to form rivets, bolts and the like. These lubricants clogged the dies and cause the production of imperfect work-pieces.

15 The wire and rods manufactured according to this invention have a dry lubricating coating that remains on the metal even during and after the reworking of the wire so that it not only serves as a lubricant to protect the dies but also 20 does not clog the dies, the result being that the dies are able to produce perfectly formed work-pieces.

In carrying out this invention the wire or rods are first cleaned to remove all scale, grease and 25 other foreign matter, and then given a coating of lime and baked. The lime coated wire or rods are then drawn to final gage using a novel lubricant consisting of a mixture of aluminum stearate or other metallic stearate insoluble in 30 water, and hydrated lime, which is drawn into the die with the wire or rods. The resultant products are wire or rods having a surface comprising a fixed impregnated coating of the lubricating compound.

35 Care is taken to keep all grease or other foreign matter from coming in contact with the wire or rods after they are cleaned and prior to their being reworked.

After the wire or rods are cleaned they may, in 40 some instances, be given either a heavy or light sull coat although this is not always essential and is eliminated when particularly bright stock is desired. In order to form a sull coat the cleaned rods are kept moist for a time by means of fine 45 sprays of water. The action of this water, together with that of the oxygen of the atmosphere and traces of acid which may still be on the rods from the cleaning operation, form a coating of a faint brownish or greenish rust or sull.

50 The lime coating may be applied as either a cold light dip or as a hot heavy coating as desired.

The mixture of aluminum stearate and hydrated lime preferably used as a lubricant may be 55 mixed in various proportions according to the

results desired. For instance, the following proportions have been used to advantage:

|                   | Parts by volume |
|-------------------|-----------------|
| Aluminum stearate | 5—4—6 60        |
| Hydrated lime     | 4—5—3           |

It will be understood that I do not wish to be limited to the above proportions, however, since many other proportions may be used with good results, and other insoluble metallic stearates 65 may also be substituted for the aluminum stearate.

The wire or rods having the coating of this invention are characterized by the fact that the coating adheres to and remains an integral part 70 of the metal even after the stock has been worked by cold forging in dies to form rivets, bolts and similar articles having upset heads, extruded shanks and the like.

After the workpieces are formed from the coated wire or rods of this invention they may be 75 heat treated and the lubricating coating will then be destroyed.

While I have described one particular use for the wire and rods made in accordance with this 80 invention it will be specifically understood that I do not wish to be limited to said use, since such wire and rods may be used for many purposes wherever reworking is necessary, and also as welding electrodes and the like.

While I have described certain specific steps and sequence of steps in setting forth the above 85 practical embodiments of my invention it will be understood that I do not wish to be limited thereto since various modifications may be made without departing from the scope of my invention, as defined in the appended claims.

I claim:

1. In the manufacture of wire, rods and the like, the steps consisting of cleaning the workpiece to 95 remove all foreign matter, coating said workpiece with lime, and then drawing said lime coated workpiece through a suitable die with a lubricant consisting of a mixture of aluminum stearate and hydrated lime to reduce its gage and cause said 100 lubricant to form an impregnated coating on said workpiece.

2. In the manufacture of wire, rods and the like, the steps consisting of cleaning the workpiece to remove all foreign matter, forming a sull 105 coating on said cleaned workpiece, coating said workpiece with lime, and then drawing said lime coated workpiece through a suitable die with a lubricant consisting of a mixture of aluminum stearate and hydrated lime to reduce its gage and 110

cause said lubricant to form an impregnated coating on said workpiece.

3. In the manufacture of wire rods and the like the steps consisting of cleaning the work-piece to remove all foreign matter, coating said work-piece with lime and then drawing said lime coated work-piece through a suitable die with a lubricant consisting of a mixture of a metallic stearate insoluble in water and hydrated lime to reduce its gage and cause said lubricant to form an impregnated coating on said work-piece.

4. In the manufacture of wire rods and the like the steps consisting of cleaning the work-piece to remove all foreign matter, forming a sull 15 coating on said cleaned workpiece, coating said work-piece with lime and then drawing said lime coated work-piece through a suitable die with a lubricant consisting of a mixture of a metallic

stearate insoluble in water and hydrated lime to reduce its gage and cause said lubricant to form an impregnated coating on said work-piece.

5. A wire or rod drawing lubricant comprising a mixture of a metallic stearate insoluble in water and hydrated lime. 80

6. A wire or rod drawing lubricant comprising a mixture of a metallic stearate insoluble in water and lime.

7. A wire or rod drawing lubricant comprising a mixture of a metallic stearate insoluble in water and a calcareous material, said mixture being composed of from four to six parts by volume of the metallic stearate and of from three to five parts of calcareous material. 90

FLINT C. ELDER.

20

95

25

100

30

105

35

110

40

115

45

120

50

125

55

130

60

135

65

140

70

145

75

150